

## UNITED STATES PATENT OFFICE

2,437,995

## SELENIUM RECTIFIERS

Wayne E. Blackburn, Wilkinsburg, Pa., assignor  
to Westinghouse Electric Corporation, East  
Pittsburgh, Pa., a corporation of Pennsylvania

No Drawing. Application November 10, 1943,  
Serial No. 509,818

5 Claims. (CL 175—366)

1

My invention relates to processes of making selenium rectifiers and, in particular relates to methods of reducing the leakage current which flows through such rectifiers in their high resistance, i. e., normally non-conducting, direction.

One object of my invention is to provide a method of reducing the losses due to current-heating in selenium rectifiers.

Another object of my invention is to provide a method of reducing current flow in the high resistance direction through selenium rectifiers.

Still another object of my invention is to provide a method of increasing the resistance of selenium rectifiers to current flow in their high resistance direction without unduly increasing their resistance to current flow in their low resistance direction.

Other objects of my invention will become apparent upon reading the following description. In accordance with the preferred form of my invention, I produce selenium rectifiers by sandblasting a steel plate and thereafter nickel plating the surface. I then dip the steel plate in molten selenium and remove the selenium in excess of a thin uniform film. One convenient way of carrying out this operation is to mount the steel plates on a spindle which is dipped into the molten selenium and withdrawn therefrom while rotating, thereby causing centrifugal force to remove the excessive amounts of selenium from the surface. I then deposit a contact on the free surface of the selenium, preferably by Schoop-spraying it with cadmium.

While I have described the above process as using selenium, it may be desirable to use selenium in which has been dissolved about .1% of bromine. The above-described steps of producing selenium rectifiers are described in my copending application Serial No. 509,817, filed November 10, 1943, for Method of making selenium rectifiers. I then anneal the unit thus formed at a temperature of between 170 and 185° C., preferably for a period of at least 6 hours. The foregoing method of producing selenium rectifiers is that described in my copending application Serial No. 509,817, filed November 10, 1943, for Method of making selenium rectifiers but the following procedure is likewise applicable to rectifiers in which the annealing process is carried out before the deposition of the contact layer instead of after it.

I have found that in the case of rectifier units made by the processes just described, it is possible to reduce leakage current which tends to

2

flow through the rectifier in the high resistance, or normally non-conductive direction, by impressing between the two terminal plates a direct-current voltage having a polarity which tends to cause current flow in the high resistance direction. In order to obtain best results, it is necessary that at some time during the course of the treatment the voltage should rise to a value greater than that to which the rectifier will have to withstand in its high resistance direction during service on alternating-current supplies. The application of such a forming voltage gradually increases the resistance to leakage current and does so without causing a deleterious increase of resistance to the flow of current through the rectifier in the conductive direction.

However, I have found that if a voltage of the magnitude just described is to be applied to the rectifier, it must be done so in accordance with certain rules of procedure; otherwise the wattage dissipated during the forming process is likely to melt the contact electrode. It might appear that by sufficiently cooling the contact electrode this difficulty could be overcome, but I have found that if such cooling is resorted to, the forming operation has very little effect on the leakage current.

I have found, however, that if the temperature coefficient of resistance in the reverse direction of such rectifiers is measured, this temperature coefficient is negative up to a certain temperature of the order of 155° C. and then becomes positive. This result is further facilitated by the application of a voltage considerably below the maximum which the rectifier must stand in the reverse-current direction in service and gradually raising this voltage to a value higher than said maximum value.

One very convenient way of carrying out the above-described procedure is to apply the lower value of forming voltage just described to a rectifier which is provided with means for artificially cooling its contact layer. The amount of cooling effect is then adjusted until, with this lower value of inverse voltage applied, the rectifier comes to equilibrium at the temperature of about 155° C. It will be found that under the action of this voltage, the resistance of the rectifier gradually increases. In consequence of this increase, the heating effect of current flow grows smaller and it is necessary to raise the impressed voltage if the unit is to be maintained at a temperature of 155° C. Such an increase of voltage is accordingly made and continued preferably at such a

rate as to maintain the unit always at the above-mentioned temperature until the applied voltage becomes greater than the maximum reverse voltage that the rectifier will ever have to withstand in actual service. To take a specific example, I have found that with rectifiers made in accordance with the foregoing description, the initial voltage across a single selenium layer should be about 12 volts and the application of this voltage should be continued with increasing values until it has reached 32 volts or more.

While I have described a specific embodiment of my invention in accordance with the patent statutes, the principles thereof are of broader application in ways that will be self-evident to those skilled in the art.

I claim as my invention:

1. The process of making selenium units which comprises depositing a layer of selenium on a metallic plate, forming a contact layer on the free surface of said selenium, annealing the unit thus formed and thereafter applying a direct-current voltage across the selenium in a direction tending to send current in the high resistance direction while maintaining the temperature of said unit at about 155° C., said voltage having an initial value below the maximum which said unit must stand in the reverse current direction in service, and being gradually raised to a value higher than said maximum.

2. The process of making selenium units which comprises depositing a layer of selenium on a metallic plate, forming a contact layer on the free surface of said selenium, annealing the unit thus formed and thereafter applying a direct-current voltage across the selenium in a direction tending to send current in the high resistance direction while maintaining said unit at about the temperature at which its temperature-resistance coefficient in respect to current flow in the high resistance direction becomes positive, said voltage having an initial value below the maximum which said unit must stand in the reverse current direction in service, and being gradually raised to a value higher than said maximum.

3. The method of forming selenium rectifiers

which comprises sandblasting a steel plate, nickel plating it, dipping it while rotating into molten selenium and withdrawing it therefrom, providing a contact layer on the free surface of said selenium, annealing said unit and thereafter impressing across the selenium in its high resistance direction a direct-current voltage which is maintained at a value such that the temperature of the unit remains at about 155° C.

4. The method of electrically forming a selenium unit comprising a layer of annealed selenium sandwiched between two conducting surfaces which comprises impressing across said layer in the high resistance direction a direct-current voltage which is maintained at a value at least sufficient to insure a positive temperature-resistance coefficient in respect to current flow in the high resistance direction through said selenium.

5. The method of electrically forming a selenium unit comprising a layer of annealed selenium sandwiched between two conducting surfaces which comprises impressing across said layer in the high resistance direction a direct-current voltage which is maintained at a value which keeps the temperature of said unit at about 155° C.

WAYNE E. BLACKBURN.

#### REFERENCES CITED

30 The following references are of record in the file of this patent:

#### UNITED STATES PATENTS

| 35 | Number    | Name                 | Date          |
|----|-----------|----------------------|---------------|
|    | 2,229,807 | Hoppe et al. -----   | Jan. 28, 1941 |
|    | 2,246,161 | Ademstedt et al. --- | June 17, 1941 |
|    | 2,261,725 | Hoppe -----          | Nov. 4, 1941  |
|    | 2,279,187 | Thompson -----       | Apr. 7, 1942  |
| 40 | 2,339,613 | Becker et al. -----  | Jan. 18, 1944 |

#### OTHER REFERENCES

"Notes on Resistances of Selenium Cells Deposited in Certain Cases"; an article from the Journal of the Optical Society of America, vol. 25, No. 1, pages 1, 2 and 3, Jan. 1935.